# EUROPEAN PATENT SPECIFICATION

(11) **EP 0 010 408 B1**
(45) Date of publication and mention of the grant of the patent: **16.02.1983**
(21) Application number: 79302194.0
(22) Date of filing: 12.10.1979
(51) Int. Cl.: B24D 15/04

(54) **Method of preparing abrasive foam material**
Verfahren zur Herstellung von Schleifschaumkunststoff
Procédé pour la fabrication de matière plastique spongieuse abrasive

(30) Priority: 13.10.1978 GB 4045278
(43) Date of publication of application: 30.04.1980
(73) Proprietor: Barron, Robert Michael, Southampton SO1 2LG Hampshire (GB)
(72) Inventor: Barron, Robert Michael, Southampton SO1 2LG Hampshire (GB)
(74) Representative: Smith, Philip Antony

## Description

The invention relates to the production of an open-cell foam polymeric material with an abrasive surface, which can be used, for example, to make scouring and cleaning pads for domestic use.

FR-A-1,465,778 describes the production of such an abrasive surface on a foam sheet by the application of a hardenable resin to the surface of the sheet. The resin penetrates from the surface of the sheet so that there is a progressive decrease in hardness from the surface into the body of the foam. The hardening resin can be applied in discrete areas, for example as a pattern of circular areas separated by untreated, and therefore soft, areas of foam.

In accordance with the present invention there is provided a method of providing an abrasive surface on a sheet of compressible open-cell foam polymeric material by the application of a hardenable resin to the surface of the sheet characterized in that a stencil (11) having a multiplicity of holes (12) is arranged on the surface of the foam sheet (1µ), pressure is applied to impress the stencil into the sheet (Fig. 1), the hardenable resin is applied to the surface of the stencil remote from the foam sheet so that the resin contacts the foam sheet in the region of the holes in the stencil, the stencil is removed and the resin (14) is allowed or caused to harden.

By the use of this method the resin is incorporated into the sheet of compressible foam material in the region of the holes in the stencil and does not project from the surface of the sheet. The resin, which can contain an abrasive substance, is applied in such a way as not to fill the cells of the foam material. The resin coating thus hardens the cell structure in the regions in which it is incorporated but should not create a continuous hard surface which closes the cells at the surface. It is however likely to reduce communication between the cells of an open foam structure in the region in which it is incorporated. Since the body of the foam sheet remains unaltered it will absorb the cleaning fluid and supply it to the hardened abrasive regions.

Hence the sheet of foam material is provided with a pattern of regions of hardened resin which do not adversely affect the flexibility of the foam sheet. The resin, being impregnated in the foam material, is unlikely to become separated from the sheet of foam material. Since the resin is applied in a multiplicity of distinct regions it is less likely to crack than if applied as a continuous superficial coating.

The invention will be further described by way of example and with reference to the accompanying drawings, in which:-
Fig. 1 is a section through a sheet of compressible foam polymeric material and a stencil used in the method according to the invention; and
Fig. 2 is a section through the sheet of foam polymeric material shown in Fig. 1, provided with an abrasive surface by a method according to the invention.

In the drawings is shown a sheet of compressible foam plastics material 10 which is of the "open-cell" type in which neighbouring cells communicate with each other. The foam sheet is preferably of polyurethane although there are many alternative materials, for example various rubbers, plasticised P.V.C., modified cellulose. A typical polyurethane foam material has the following characteristics:-
Density: 15 to 45 kg/ₘ³
Hardness to B.S. 3667: 20 to 30
Elongation at break: 100 to 300%
Tensile strength: 69 to 138 kPa (10 to 20 p.s.i.)
Cell Diameters: 0.25 to 2.00 mm

The thickness of the sheet is preferably in the range from 2 mm to 50 mm.

To provide the sheet of foam material 10 with an abrasive surface, a stencil 11 having a multiplicity of holes 12 in a regular pattern is arranged against a surface of the sheet and pressure is applied to the stencil to impress it into the sheet as shown in Fig. 1. The stencil 11 is made of a rigid material, for example a metal or a rigid plastics material, and its thickness is typically in the range 0.5 to 2.0 mm through this dimension is not critical. The holes 12 can be of any shape but for convenience will usually be circular and have diameters approximately in the range 2 to 10 mm, or perhaps up to 15 mm. A typical example has circular holes of 8 mm diameter at 12 mm spacing between centres.

Hence the holes have an area approximately in the range 3 to 150 but preferably less than 80 square mm. It will be appreciated that the area of one hole in the stencil is small compared to the area of, for example, a scouring pad for domestic use, which is one of the articles which can be produced directly from the finished sheet of abrasive foam material. The total area of the holes 12 is preferably between 25 and 60% of the total area of the stencil. However if the shape of the holes approximates to a square or rectangle it is possible to increase the total area of the holes to as much as 90% of the total area of the stencil.

Sufficient pressure is applied to the stencil 11 to ensure that foam material protrudes through the holes 12 and projects from the opposite face of the stencil as shown in Fig. 1.

A hardenable liquid resin is applied to the stencil 11 and spread over the stencil by means of a rigid spreader member, for example a metal or hard rubber blade. The resin preferably comprises an epoxy resin and an example of the constituents of a suitable resin is as follows:-

DER 321 is a product of the Dow Chemical Company available through Casa Chemicals Ltd. "Synolide 960" is a product of General Mills Corpn. available from Cray Valley Products Ltd. 200 mesh is a sieve size which passes particles of up to 75 µm diameter.

Other resins may be used depending on the intended use of the finished abrasive foam sheet and examples of alternative resins are natural and synthetic rubbers, acrylics, P.V.C., and phenolformaldehyde resins. Similarly the amount and type of abrasive filler used can be varied and resins containing no abrasive filler can be used.

As the spreader member is drawn across the stencil 11 it comes into contact with the foam material where it protrudes through the holes 12, and smears resin into the material. The stencil 11 is then removed from the sheet of foam material 10 which is then exposed to conditions suitable for hardening the resin associated with the sheet. To harden the example of a resin described above, the sheet should be heated to 125°C for about 5 minutes.

Fig. 2 shows the material produced by this method. The sheet of foam material 10 is provided with an abrasive surface 13 comprising a multiplicity of distinct regions of hardened resin 14 corresponding to the holes 12 in the stencil 11. The resin is incorporated into the sheet of material 10 and does not substantially project above the surface of the sheet. This is due to the compression of the material by the stencil and the working of the resin into protruding areas of foam material as they are engaged by the spreader member. In addition, when the stencil is removed the foam material expands and, since the material is of the "open-cell" type, the liquid resin is drawn into the sheet from cell to cell with the result that, in general, the cells which contain resin are not filled by the resin but have the cell walls coated. The cell structure is thus retained, which is important for the cleaning action of the product. The cell diameters are preferably in the range 0.25 to 2.0 mm.

As can be seen in Fig. 2, the resin is incorporated in the cells of the foam material and in use of a part of the sheet, for example as a scouring pad, the resin is much less likely to get separated from the foam material than if it is applied as a superficial coating. A continuous superficial coating of resin is also prone to splitting, which does not occur if resin is applied in a pattern of distinct small regions. The surface structure of the cells of the foam sheet, within the regions of hardened resin 14, contributes an abrasive effect, as does the discontinuity of the resin-impregnated regions and the presence of any abrasive material in the resin.

Products made using very thin section polyurethane foams (i.e. 2-5 mm) are too weak and dimensionally unstable to be durable. Such foams can, however, be easily modified and strengthened by lamination to a lightweight fabric (e.g. cotton or synthetic), either woven or non-woven. These fabrics would have weights of 20-100 g/m². A further improvement in strength occurs during the coating/printing process, as the liquid resin will completely penetrate the thin foam and adhere to the fabric laminated to the back of the foam.

The resulting product can either be used as an abrasive or cleaning cloth, or further laminated to blocks of polyurethane or other rigid foams and cut up into pads.

Since the structure of the foam and nature of the polymer constituting the foam are retained during the printing and hardening process, the eventual durability of the product is dependent upon the strength of the particular foam used. Therefore, when the cheapest polyurethane foams are used, they are found to be less durable than the better quality foams. However, it has been found that useful products of good durability can be made from the cheapest, lightest density polyurethane foams if a thin film of thermoplastic resin is fused onto the abrasive surface. This film strengthens the foam surface considerably and does not interfere too much with the abrasive properties of the hardened areas on the working surface.

Typical films are: poly(ethylene), poly(ethylene vinyl acetate), plasticised poly(vinyl chloride) and its copolymers, natural rubber - hydrochloride, etc.

Film thicknesses are typically 25-50 microns.

The film is fused to the foam surface at 120-160°C for 5-20 seconds at about 2 kg/cm² depending upon the particular film used and thickness of the coated foam.

It will be appreciated that cleaning or scouring pads can be made from a sheet of abrasive foam material according to the invention simply by cutting the sheets into pads of a suitable size for the intended use. Sheets having differing abrasive characteristics may be produced as described above. Cleaning or scouring pads cut from a sheet of abrasive foam may be used to clean, for example, cooking utensils, baths, kitchen sinks, paintwork, and vehicle windscreens. For these purposes they must be used with a liquid, for example water.

## Claims

1. A method of providing an abrasive surface on a sheet of compressible open-cell foam polymeric material by the application of a hardenable resin (14) to the surface of the sheet characterized in that a stencil (11) having a multiplicity of holes (12) is arranged on the surface of the foam sheet (10), pressure is applied to impress the stencil into the sheet (Fig. 1), the hardenable resin is applied to the surface of the stencil remote from the foam sheet so that the resin contacts the foam sheet in the region of the holes in the stencil, the stencil is removed and the resin (14) is allowed or caused to harden.

2. A method as claimed in claim 1, wherein the holes (12) in the stencil (11) are circular holes having a total area of between 25% and 60% of the total area of the stencil.

3. A method as claimed in claim 1 or 2, wherein the pressure applied to the stencil (11) is sufficient to cause the foam material to project from the face of the stencil remote from the foam sheet.

4. A method as claimed in any of claims 1 to 3, in which the resin is hardened by heating of the foam sheet after removal of the stencil.

5. A method as claimed in any preceding claims, in which the foam sheet is initially laminated with a fabric backing sheet and is of such thickness that the hardenable resin passes through the foam sheet and bonds to the backing sheet.

6. A method as claimed in any of the preceding claims in which after hardening of the resin a thin film of thermoplastic resin is fused to the surface of the sheet carrying the hardened resin regions.

## Revendications

1. Procédé pour ménager une surface abrasive sur une feuille en une matière polymère mousse à cellules ouvertes compressible par l'application d'une résine durcissable (14) à la surface de la feuille, caractérisé en ce qu'il consiste à disposer un pochoir (11) ayant une multiplicité de trous (12) sur la surface de la feuille mousse (10), à appliquer une pression pour imprimer le pochoir dans la feuille (figure 1), à appliquer la résine durcissable la surface du pochoir qui est éloignée de la feuille mousse de manière à ce que la résine vienne en contact avec la feuille mousse dans la région des trous du pochoir, à enlever le pochoir et à laisser durcir ou à provoquer le durcissement de la résine (14).

2. Procédé suivant la revendication 1, caractérisé en ce que les trous (12) du pochoir (11) sont des trous circulaires ayant une surface totale représentant de 25 à 60% de la surface totale du pochoir.

3. Procédé suivant la revendication 1 ou 2, caractérisé en ce que la pression appliquée au pochoir (11) est suffisante pour que la matière mousse fasse saillie de la face du pochoir éloignée de la feuille mousse.

4. Procédé suivant l'une quelconque des revendications 1 à 3, caractérisé en ce qu'il consiste à durcir la résine en chauffant la feuille mousse après enlèvement du pochoir.

5. Procédé suivant l'une quelconque des revendications précédentes, caractérisé en ce que la feuille mousse est plaquée initialement à l'aide d'une feuille de renforcement en tissu et a une épaisseur telle que la résine durcissable traverse la feuille mousse et se lie à la feuille de renforcement.

6. Procédé suivant l'une quelconque des revendications précédentes qui consiste, après avoir durci la résine, à faire fondre une mince pellicule de résine thermoplastique à la surface de la feuille portant les régions de résine durcies.

## Patentansprüche

1. Verfahren zur Aufbringung einer schmirgelartigen Oberfläche auf eine Bahn aus zusammendrückbarem, offenzelligem Schaumstoffpolymerisat durch Aufbringung eines härtbaren Harzes (14) auf die Oberfläche der Bahn, dadurch gekennzeichnet, daß man auf die Oberfläche der Schaumstoffbahn (10) eine Schablone (11) mit einer Vielzahl von Löchern (12) aufbringt, die Schablone in die Bahn durch Anwendung von Druck eindrückt (Fig. 1), danach das härtbare Harz auf die der Schaumstoffbahn abgewandte Oberfläche der Schablone aufbringt, so daß das Harz die Schaumstoffbahn im Bereich der Löcher in der Schablone berührt, die Schablone entfernt und das Harz (14) aushärten läßt.

2. Verfahren gemäß Anspruch 1, dadurch gekennzeichnet, daß man die Löcher (12) in der Schablone (11) als kreisförmige Löcher ausbildet, die eine Gesamtfläche von 25 bis 60% der Schablonenberfläche ausmachen.

3. Verfahren gemäß Anspruch 1 oder 2, dadurch gekennzeichnet, daß man auf die Schablone (11) einen Druck ausübt, der ausreicht, um das Schaumstoffmaterial von der der Schaumstoffbahn abgewandten Seite der Schablone hervortreten zu lassen.

4. Verfahren gemäß einem der Ansprüche 1 bis 3, dadurch gekennzeichnet, daß man das Harz durch Erhitzen der Schaumstoffbahn nach Entfernung der Schablone aushärtet.

5. Verfahren gemäß einem der vorhergehenden Ansprüche, dadurch gekennzeichnet, daß man die Schaumstoffbahn zunächst mit einem Stützgewebe laminiert und die Dicke der Schaumstoffbahn derart wählt, daß das härtbare Harz die Schaumstoffbahn durchdringt und sie mit dem Stützgewebe verbindet.

6. Verfahren gemäß einem der vorhergehenden Ansprüche, dadurch gekennzeichnet, daß man nach dem Aushärten des Harzes eine dünne Schicht aus thermoplastischem Kunststoff auf die Oberfläche der Bahn, die die Bereiche mit dem ausgehärteten Harz aufweist, aufschmilzt.
